

# UNITED STATES PATENT OFFICE.

HILLIARY ELDREDGE, OF NEW YORK, N. Y., ASSIGNOR, BY MESNE ASSIGNMENTS, TO  
THE METALS PLATING COMPANY, A CORPORATION OF NEW JERSEY.

## PLATING FERROUS METALS.

1,197,616.

Specification of Letters Patent. Patented Sept. 12, 1916.

No Drawing.

Application filed April 3, 1913. Serial No. 758,536.

To all whom it may concern:

Be it known that I, HILLIARY ELDREDGE, a citizen of the United States, residing at the city of New York, borough of Richmond, in the county of Richmond and State of New York, have invented certain new and useful Improvements in Plating Ferrous Metals, of which the following is a specification.

10 My invention relates broadly and generally to new and useful methods for coating or plating ferrous metals with copper, or other non-ferrous metal or metals, (that is to say, iron or steel, or alloys whose chief 15 constituent is iron) or alloys thereof, having less affinity for oxygen than ferrous metals, and to new and useful articles of manufacture produced thereby.

In proceeding according to my invention 20 I subject the ferrous metal to be plated or coated while in surface contact with an oxid of the non-ferrous plating metal, to a temperature sufficient to convert the oxid of the plating metal into metal.

25 I will now proceed to describe some of the various methods which may be employed in carrying my invention into effect:

If it is desired to coat a body of ferrous metal with a plating of metallic copper, 30 I may apply to the surface of the ferrous metal, say, sheet-iron, a thin coating of copper oxid, preferably cupric oxid ( $CuO$ ). I may use cuprous oxid ( $Cu_2O$ ), but prefer the cupric oxid as being cheaper and giving better results. This coating may be applied in a number of ways without departing from the spirit and scope of my invention, but I prefer to apply it in the form of a mixture of cupric oxid with a suitable 35 liquid vehicle which may be prepared by mixing equal parts by weight of the cupric oxid and water. This mixture may then be applied to the ferrous body in any suitable way and as evenly as possible. The

40 ferrous metal coated as above described, is then placed in a furnace or muffle and subjected to a degree of heat sufficient to convert the copper oxid into copper. I have found that, in order to produce the best 45 results, the temperature to which the coated metal is subjected, in the case of copper, should be at or about the melting point of copper.

The ferrous metal with the copper oxid

coating is subjected to the degree of heat 55 mentioned above until the desired reaction described takes place, after which the metal should be promptly removed from the furnace or muffle because further exposure to the heat is unnecessary. The period of time 60 to the desired temperature depends largely upon the thickness of the ferrous metal, for instance with No. 30 sheet iron, which is 65  $12\frac{1}{2}$  one-thousandths of an inch in thickness, the period of subjection to the heat is approximately four (4) or five (5) to ten (10) seconds, and it will be understood that metal of less thickness will require a less time, and metal of greater thickness 70 will require more time. It will be understood that I do not limit myself to the exact period stated, but give the same as one which will be proper for No. 30 sheet iron. Upon the removal of the ferrous metal from 75 the furnace or muffle and cooling, said ferrous metal will be found to be covered with a closely adherent continuous plating of copper next thereto, which layer of copper is covered by a superposed continuous layer 80 of oxid of iron. This layer of oxid of iron may be removed by a suitable solvent (such as hot weak sulfuric acid, for example), or by exposing it to the action of a reducing gas, or by abrasion, or other suitable procedure.

The manner I have described above for coating the oxid of the non-ferrous metal suspended in a liquid onto the iron, is especially adapted to the plating of thin, flat 90 metal bodies, such as sheet iron or sheet steel. For applying the oxid of the non-ferrous metal to heavy bodies, such as angle iron and structural iron and steel elements, I may apply the oxid of the coating metal to 95 the ferrous body while the latter is in the furnace, by sifting the finely-divided copper oxid upon the body in any suitable manner. When this method of applying the copper oxid is employed, the iron may first 100 be heated in the furnace to, say,  $1100^{\circ}$  to  $1200^{\circ}$  C. (that is, from a yellow to a beginning white heat), before the oxid is sifted thereon. Or, the iron, after being heated to the required temperature, may be 105 withdrawn from the furnace and the copper oxid then sifted upon it. Under these circumstances the reaction may take place out-

side the furnace. If it does not take place outside the furnace, the body should be returned to the furnace and heated.

In all of the examples given, it will be understood that in order to produce the best results, the duration during which the ferrous metal is subjected to a desired temperature, namely at or about the melting point of copper, is approximately from 4 or 5 seconds to 10 seconds, but it will be understood that it may be less or greater, and that it must be long enough to allow the copper to be reduced and to adhere as a non-stripping plate to the surface of the iron.

While the methods of procedure described are particularly adapted for the plating of ferrous metal with copper, they can be advantageously used in coating ferrous metal with lead, or silver, or other metals having less affinity for oxygen than has iron. With these other plating metals, as with copper, the process should be carried out at temperatures likewise as high as but not too far above the melting point of the oxid of the plating metal. I have also found that plating of alloys with superposed layer of resulting oxid, may, in manners similar to those above described, be made upon the bodies of ferrous metal, as, for instance, I can apply a plating of bronze by using a mixture of cupric oxid (CuO), and tin oxid (SnO), in definite proportions to produce the desired bronze, or a plating of lead and copper may be produced.

What I claim and desire to secure by Letters Patent of the United States is:—

1. The method of plating ferrous metal, which consists in subjecting the same while in surface contact with an oxid of a metal having less affinity for oxygen than has iron, to a temperature sufficient to effect reduction of the oxid to metal in a substantially continuous coating over the ferrous metal into a weld-like union therewith, and producing a coating of oxid of iron superposed on the plating metal, and subsequently removing the oxid of iron.

2. The method of plating ferrous metal, which consists in subjecting the same while in surface contact with an oxid of a metal having less affinity for oxygen than has iron, to a temperature approximating the melting point of the oxid for a period sufficient to effect reduction of the oxid to metal in a substantially continuous coating over the ferrous metal into a weld-like union therewith.

3. The method of plating ferrous metal, which consists in subjecting the same while in surface contact with an oxid of a metal having less affinity for oxygen than has iron, to a temperature approximating the melting point of the oxid for a period of from approximately four (4) seconds to approximately ten (10) seconds after the desired temperature is reached, and thereby causing reduction of the oxid of metal in a substantially continuous coating over the ferrous metal into a weld-like union therewith.

4. The method of plating ferrous metal with copper which consists in coating ferrous metal with an oxid of copper, and subjecting the same to heat at substantially the melting point of the oxid of copper until the iron reacts with the oxygen of the oxid to form a layer of metallic copper upon the iron.

5. The method of plating ferrous metal with copper, which consists in coating the ferrous metal with cupric oxid, and subjecting the same to heat at substantially the melting point of said oxid until the iron reacts with the oxygen of the oxid to form a layer of metallic copper upon the iron.

6. The method of plating ferrous metal, which consists in applying to the ferrous metal a liquid coating in which is suspended an oxid of a metal having less affinity for oxygen than has iron, and subjecting the same to a temperature approximately the melting point of the oxid for a period sufficient to effect reduction of the oxid to metal in a substantially continuous coating over the ferrous metal into a weld-like union therewith.

7. The method of plating ferrous metal, which consists in coating the same with an oxid of a metal having less affinity for oxygen than has iron, and subsequently subjecting the coated ferrous metal to a temperature sufficient to effect reduction of the oxid to metal in a substantially continuous coating over the ferrous metal into a weld-like union therewith, and producing a coating of oxid of iron superposed on the plating metal, and subsequently removing the oxid of iron.

In testimony whereof I have hereunto signed my name in the presence of two subscribing witnesses.

HILLIARY ELDRIDGE.

Witnesses:

W. S. ROCKEY,  
GEORGE C. HALL.